

A. E. GREENE.

PROCESS OF PRODUCING ALLOY STEEL.

APPLICATION FILED JAN. 6, 1909.

1,034,786.

Patented Aug. 6, 1912.

Fig. 2.



Fig. 4



Fig. 1



Witnesses:

McLellan & Young.  
Alfred Atmore

Inventor:

Albert E. Greene,  
By Barton Folk.  
Attn: 5.

# UNITED STATES PATENT OFFICE.

ALBERT E. GREENE, OF CHICAGO, ILLINOIS, ASSIGNOR TO AMERICAN ELECTRIC SMELTING AND ENGINEERING COMPANY, OF ST. LOUIS, MISSOURI, A CORPORATION OF MISSOURI.

## PROCESS OF PRODUCING ALLOY STEEL.

1,034,786.

Specification of Letters Patent. Patented Aug. 6, 1912.

Application filed January 6, 1909. Serial No. 470,921.

To all whom it may concern:

Be it known that I, ALBERT E. GREENE, citizen of the United States, residing at Chicago, in the county of Cook and State of Illinois, have invented a certain new and useful Improvement in Processes of Producing Alloy Steel, of which the following is a full, clear, concise, and exact description.

10 My invention relates to the production of alloys in general and more particularly to manganese iron alloys, especially, in this latter case, to the production of low-carbon manganese-steel.

15 In one of its aspects my invention contemplates the production of alloy-steels in which the alloying metal or metals consist of any one or more of the following, namely, titanium, silicon, nickel, cobalt, 20 molybdenum, tungsten, chromium and the like.

25 The process of my invention has for its object in general the production, in a rapid and efficient manner, of alloys free to the desired degree from such impurities as carbon, silicon, sulfur, phosphorus, etc.

30 In the case of iron alloys the process has for its object more particularly the production of the type of alloys known as steel, approximately free from phosphorus and sulfur and having their content of carbon regulated as desired from a maximum to a minimum, while retaining in the alloys any of the aforementioned metals that may be 35 desired to retain therein.

35 The processes now in general use for producing alloy steels are based on the addition of a low-carbon ferro-alloy to the desired grade of steel and thus producing the 40 alloy-steel. For example, manganese-steel is commonly produced by adding low-carbon ferro-manganese to ordinary steel while the latter is in a molten condition. In the production of such low-carbon ferro-alloys it 45 has heretofore been found easier to reduce the oxids of the metals with an excess of carbon, either in a blast furnace or in an electric furnace, and then to refine the resultant product, containing an excess of car-

50 bon, to produce the low-carbon ferro-alloy. The refining operation has been either by the Bessemer process or else by an electric furnace process. These processes are un-

satisfactory for the reason that they are costly and inefficient.

55 The refining by the Bessemer process has the inherent objection of lack of temperature regulation, resulting in an inefficient control of the process. Moreover in such refining process the metal to be refined itself suffers loss by oxidation. For these reasons the refining by such process of alloys of iron with such metals as manganese and nickel to produce an alloy-steel has even been found impossible. It has in general been found more economical for the production of low-carbon alloy-steels to produce a refined high per cent. alloy and add this to the refined steel in such proportions as to give the desired product.

60 In refining alloys of the more refractory metals like chromium, tungsten, titanium, etc., which it is more economical to treat in an electric furnace, difficulties have been experienced in the elimination of the excess of carbon, such elimination requiring considerable length of time with a resultant increase in cost, and also in certain cases being attended with a loss of the desired metals themselves by oxidation.

65 My invention contemplates the production of the refined steel or other alloy directly from the ore or from the product of the blast furnace, as may be deemed desirable, in the case of the more easily reducible metals, and in the case of alloys of the more refractory metals to produce such alloy in concentrated form free from impurities. So far as I am aware, it is new, as contemplated by the process of my invention, to produce manganese-steel directly from the ore or from the product of the blast furnace.

70 In producing my process I start with the ore itself or with the blast furnace output, containing the metals which enter into the alloy, which material ordinarily contains such impurities as carbon, silicon, sulfur and phosphorus, and to remove any or all of such impurities to the desired degree, while retaining in the bath the metal which 75 it is desired to alloy with the iron to produce the alloy-steel.

75 The process of my present invention is in general similar to the process set forth in my co-pending applications Serial Number 105 444,740, filed July 22nd, 1908 and Serial

Number 488,360, filed April 7, 1909. It is based upon a combined regulation of the furnace temperature and of the pressure of dissociation of the active constituent or constituents of the gaseous agent employed for producing reactions in the molten material under treatment.

My invention further consists in regulating the temperature and actual pressure in the furnace chamber in which the material is being treated in such manner that volatilization of the metals forming the alloy is lessened or prevented, and in meanwhile blowing the bath with a gas having a pressure of dissociation or partial pressure suitable for effecting desired reactions in the bath.

The several features of my invention will be hereinafter set forth in detail.

The process is preferably carried out in a type of electric furnace in which the concentration of high temperatures at one or more points is avoided, since such concentration of temperatures is liable to cause a volatilization of the volatizable elements of the bath. While the practice of this process is not confined to any particular type of furnace, and though a Heroult or Girod furnace may be employed, I preferably practise this process in connection with an induction furnace or other furnace in which the bath is uniformly heated throughout and preferably use a furnace without carbon electrodes whenever the carbon is not desired in the alloy. In the accompanying drawings two such types of furnaces are shown.

In said drawings, Figure 1 is a sectional view of an electric furnace on the line 1—1 of Fig. 2, showing one type of furnace with which my invention may be practised. Fig. 2 is a sectional view on the line 2—2 of Fig. 1. Fig. 3 is a vertical section of an induction furnace with which the process may be practised; and Fig. 4 is a plan view of the furnace shown in Fig. 3.

Similar reference characters are used to designate similar parts wherever shown.

Referring to Figs. 1 and 2 the steel casting 1 of the furnace is supported from trunnions 2, 3, in order that the furnace may be tilted in the usual manner. The side walls 4 are made of refractory material, and the crucible 5 is provided with a removable top 6 of silica or other suitable material. Electrodes 7, 7 extend through the side walls of the furnace and dip through the slag 8 into the metal 9 of the bath. However, by tilting the furnace, the electrode on one side of the furnace can be made to dip only into the slag, and the electrode on the other side into the molten metal. By thus causing the electrodes to dip into the bath, the formation of an arc is avoided, this being desirable for the reason that the high temperature of the arc concentrated at one or more points

is likely to cause a volatilization of certain volatilizable elements which it may be desirable to retain in the metal. Since the electrodes dip into the bath, a current of low voltage and high amperage is employed, and the current may be regulated by varying the voltage. Either direct or alternating current may be employed, but in some cases I preferably employ direct current to assist by electrolysis the reduction of the metallic oxids. The trunnion 2 is hollow to provide a passage 10 communicating with the twyler pipe 11. Twylers 12, 12 extend downward through the wall 4 (see Fig. 2). The blowing gas is introduced under pressure through the passage 10 to the twylers 12 in the usual manner. Said twylers are inclined downward in order that the gas may be more thoroughly blown into the bath. The exhaust gas is preferably led out through the exhaust pipe 13, since such gases are ordinarily collected on account of their value.

Figs. 3 and 4 show a well-known type of induction furnace. The steel casing 14 thereof may be supported in any suitable manner. The walls 15 inclosed in said casing are annular in shape and surround one leg of the transformer core 16. Said core is wound with one or more coils 17, which serve as the primary of the transformer, the secondary thereof consisting of the metallic bath 18 contained in the furnace chamber 19. The voltage impressed on the primary of the induction furnace may be varied at will, thereby regulating the temperature of the bath. The chamber 19 is provided with a cover, which is preferably made in a plurality of sections 20. Gas is admitted from the gas main 21 and the flow thereof is controlled by the valve 22. The twylers 23 which are connected by means of pipes 24 with the gas main extend through the cover 20. The exhaust gas passes out through exhaust gas pipe 25.

In certain cases, as will hereinafter more fully appear, the process may be advantageously expedited by controlling the pressure in the furnace chamber. I may, therefore, employ a suction fan 26 for removing the exhaust gases as formed through the exhaust pipe 25, thus maintaining the atmosphere within the chamber under a reduced pressure. While the twylers are shown as directing the gas down upon the surface of the bath, any well known arrangement of twylers for introducing the gas into the bath may be substituted for the arrangement shown. In practice I work at a temperature as slightly as is practicable above the melting point of the material under treatment, as for example, 1500° C. to 1600° C., in the case of manganese alloys. To remove the oxidizable impurities the molten bath is blown with a gas having an oxygen pressure at said temperature which renders it an oxidizing agent.

with respect to the impurity or impurities which it is desired to eliminate by oxidation, but which acts as a non-oxidizing or even a reducing agent with respect to the metals which it is desired to retain in the bath. In the treatment of alloys containing manganese, at the aforementioned temperatures and with a gas containing 14% of  $\text{CO}_2$  and 18% of  $\text{CO}$ , carbon can be reduced to about .03% to .05% without oxidation of the metals of the bath. For further diminution of carbon I may in some cases employ a gas containing a small amount of oxygen, as for example steam ( $\text{H}_2\text{O}$ ) and air or a hydro-carbon mixed with air, and obtain a low oxygen pressure by operating the pump 26 to reduce the pressure in the furnace chamber, thus aiding in the removal of carbon as a compound with oxygen. This method of expediting the action by reducing the pressure on the bath of the gases escaping therefrom is especially applicable to cases in which the metal or metals to be reduced are volatile only at a high temperature, as for example titanium. It will be understood, therefore, that the character of the charge and the degree of elimination desired must be taken into consideration in determining the temperature, total pressure of the gas, the active constituent of the gas, and the oxygen pressure thereof. For example, where excessive pressure conditions are desirable in order to diminish vaporization of the volatile metal, I avoid contaminating the metal with nitrogen by substituting water or hydro-carbon or products resulting from the desired reactions for nitrogen in the gaseous mixture. The requisite pressure of oxygen in the gaseous mixture may be obtained without the presence of nitrogen by substituting therefor steam together with a reducing gas, as for example carbon monoxid or hydrogen. This might be done by mixing with water gas (as for example a gas containing by volume 45%  $\text{CO}$ , 45%  $\text{H}_2$ , and 4%  $\text{CO}_2$  and traces of nitrogen), a suitable amount of carbon dioxid, steam or other oxygen containing gas to give the desired oxygen pressure. Furthermore, in treating metals which have a strong affinity for carbon, and which reduce carbon from carbon containing gases, as does chromium, I employ an oxidizing gaseous mixture of the proper oxygen pressure free from carbon compounds. In such event the desired partial pressure of the oxygen can be obtained, for example by diluting oxygen or air or steam with a reducing gas, such as hydrogen, not containing carbon.

Where sulfur and phosphorus are present, I melt with the bath a calcium or other alkaline earth containing flux to slag off these impurities. In such case the treatment of the material by the above described selective oxidation process will eliminate the oxidizable

impurities without oxidizing the metals of the bath, and since the slag is thus kept practically free from metallic oxids, as for example iron oxid, it will also readily take up the sulfur as a slag. 70  
I prefer to remove the carbon or other oxidizable impurity in the manner described herein, and then to blow the bath with a gas having less oxidizing and more reducing properties, as I have found that such subsequent treatment results in a further removal of sulfur and phosphorus. 75  
There are several advantages resulting from conducting all the operations on the product of the blast furnace in the electric furnace, rather than first treating it in an ordinary converter to remove the carbon and then continuing the treatment in the electric furnace. 80 Some of these advantages are as follows: (1) All the heat generated is saved; 85 (2) the carbon monoxid generated during the removal of the carbon reacts with the slag and causes conditions favorable to the removal of sulfur and phosphorus; (3) the slag is heated during the process of removing the carbon by what would otherwise be waste heat; and (4) the temperature can at all stages of the process be readily controlled. 90  
Having set forth in a general way the 95 variable conditions to be regulated in carrying out the process of this invention in its several applications, I will now describe one of its specific applications to the production of low-carbon manganese-steel. A charge 100 consisting of a molten spiegeleisen or other form of ferro-manganese containing such proportion of manganese as will give the desired percentage of that metal in the resulting steel is introduced into the crucible of an electric furnace, preferably an induction furnace such as shown in Figs. 3 and 4 of the drawings. Close temperature regulation is essential in order to avoid volatilization of the manganese by excessive heat. 105 I have found that a temperature of approximately  $1500^{\circ}$  C. may be maintained without excessive volatilization of manganese; and that by selecting suitable gaseous mixtures the several reactions necessary to refine the 110 material may be brought about at said temperature. A flux consisting of burned lime, calcium fluorid, or other alkaline earth composition, is added in sufficient quantities to slag the sulfur and phosphorus as sulfid, 115 and phosphid, respectively. The amount of flux should be slightly in excess of the theoretical proportions necessary to slag the impurities, as, for example, where lime is used about fifty pounds of lime per ton of 120 metal. 125  
The bath maintained at the temperature above stated is blown with a gas having the required oxygen pressure for oxidizing the carbon without oxidizing the iron or the 130

4  
 manganese. For example, blast furnace gas containing approximately 20% of carbon dioxide, 10% of carbon monoxid, and the remainder of nitrogen, hydrogen, etc., will give a satisfactory removal of carbon, silicon, sulfur and phosphorus without lessening the content of iron and manganese. If an especially complete elimination of sulfur and phosphorus is desired, the gaseous mixture is changed toward the end of the above-described blow to one containing a higher percentage of reducing gas, for example, to a gaseous mixture containing 40% of carbon monoxid, 40% of hydrogen and the remainder of nitrogen, carbon dioxid, or hydrocarbons.

While close regulation is essential, I do not wish it to be understood that any particular temperature is essential. The regulation referred to is a combined regulation of temperature and pressure of dissociation, as set forth in my aforementioned application for Letters Patent. Thus, for example, if it be desired to retain manganese in the metal, while removing sulfur and phosphorus, such result may be satisfactorily obtained by maintaining the bath at a uniform temperature of approximately 1750° C., and blowing said bath with a gas having an oxygen pressure of approximately 40 millimeters of mercury. A gas having this oxygen pressure may contain approximately 12 per cent. of CO<sub>2</sub>, 23 per cent. of CO, and the remainder of some inert gas like nitrogen or steam. A pressure of approximately 20 pounds should be maintained to lessen volatilization. The use of such a gas at the temperature mentioned causes no oxidation of the manganese, while it gives a satisfactory removal of sulfur and phosphorus. However, if the oxygen pressure of the gas be increased to 140 millimeters, the use of such gas at the temperature of 1750° C. will result in the entire elimination of the manganese.

To lessen the loss of the metal or alloy by volatilization I preferably work at a comparatively low temperature and use a gaseous mixture having a correspondingly low oxygen pressure in order to oxidize the carbon without oxidizing either the manganese or the iron.

The application of the process to the production of the other alloy-steels hereinbefore mentioned is in general similar to that just described in detail with respect to manganese steel. A brief statement of the conditions desirable in the application of the process to the production of such other alloy-steels will therefore suffice. Silicon steel containing approximately 3.25% of silicon, 0.5% of manganese, 0.2% of carbon may be produced from a charge of pig iron containing, for example 3.5% of silicon, and 0.6% manganese. The molten pig iron is

5 poured into an electric furnace provided with twyers, and the temperature of the bath is raised electrically to about 1500° C. Slag is preferably melted on top of the bath. Such slag may consist of lime and silica in approximately equal proportions. The molten bath of iron is blown with a gaseous mixture containing approximately 15% of CO<sub>2</sub> and 12% of CO, and the remainder of some inert gas, such as nitrogen. This treatment will remove the carbon and leave practically all the silicon and the manganese in the bath. Test samples of the metal after the blow is nearly completed serve to determine when the carbon is low enough. If the silicon content is too high when the carbon is down to specification, lime may be added, and the heat continued. This will rapidly take the silicon down.

10 In the application of my process to a titanium-iron alloy to make titanium steel I proceed almost in the same manner as for silicon steel. Titanium may be reduced with the iron in the blast furnace and by proceeding as described above, but using a very acid slag preferably consisting entirely of SiO<sub>2</sub> and maintaining a temperature of about 1650° C., the carbon may be eliminated while the titanium is retained. In the production of nickel steel and cobalt 15 steel a slag is preferably maintained on top of the bath, and the temperature, especially for low carbon nickel steel, is maintained somewhat higher than for manganese steel, that is, at about 1550° C. for nickel steel to contain 20% carbon. The gas is preferably made more reducing, for example, it might contain 20% CO and 15% CO<sub>2</sub>. Thus a charge of molten nickel pig iron containing 3% nickel and 4% carbon may be 20 converted directly into nickel steel. It is preferable with this steel to provide a lime slag.

25 In the manufacture of tungsten steel and molybdenum-steel or tungsten-molybdenum-steel, or steels containing either of these elements and chromium, I prefer to use an acid lined electric furnace. After providing a molten bath of the metal to be refined containing such elements, a slag is provided 110 consisting largely of silica. A temperature of about 1550° C. is maintained if the tungsten, molybdenum, or chromium does not exceed 20%, and the bath blown with a gas containing about 20% CO and 10% CO<sub>2</sub>. This will give a satisfactory elimination of carbon with a minimum loss of the metal. In refining such alloys containing more than 20% of the alloying metals, I prefer to use water gas containing 20 to 30% of hydrogen and 10 to 12% CO<sub>2</sub>. In such use, I maintain the temperature above 1700°.

30 When refining ferro-chrome, containing high percentage of chromium, of its carbon, for example to refine a 65% chromium-130

iron alloy containing 7% carbon to one containing .5% carbon, the ferro-chromium, under a straight lime slag, is blown with water gas, the bath being meanwhile raised to a temperature of at least 1750° C. to avoid the reaction between CO and chromium (Cr.). If the temperature is maintained high enough the chromium will not take up carbon from the CO. The water gas should analyze approximately 8% H, 10% CO<sub>2</sub>, 5% H<sub>2</sub>O and 10% CO and the rest nitrogen with the exception of small amounts of other hydrocarbons. In case acid elements are desired in the steel they may be retained in the molten metal by increasing the reducing conditions and making the slag more acid. If it is desired to remove silicon from a bath of steel without loss of manganese or iron, the slag may be made highly basic, for example, largely lime with a little fluor spar. By blowing the bath with a gas containing 20% CO and 12% CO<sub>2</sub>, neither the iron or manganese are oxidized but the silicon may be rapidly taken up by the slag. If it is desired to retain silicon the slag is made acid and with the same gas as just described, the silicon will be retained.

It is to be understood that I may practice the process of this invention in a continuous manner, as described for the treatment of ores in my co-pending application Serial Number 426,334, filed April 10, 1908. In such case the charge is smelted and reduced in the upper part of the blast furnace shaft, and the refining takes place in the crucible at the base of the furnace. The result of such procedure would be to keep from reduction undesirable elements and then to remove them in a slag instead of oxidizing them.

The words "high carbon" and "low carbon" as here used are relative terms, and are not intended to specify any particular percentage of carbon.

I claim:

1. The process of producing low-carbon alloy-steel, which consists in first producing a ferro-alloy high in carbon and containing the desired proportion of the alloying metal with respect to iron, maintaining the product in a molten condition at an approximately uniform elevated temperature in a refining chamber, and then subjecting the same to the action of a gaseous reagent having a pressure of disassociation suitable for the action of said reagent on an element or elements which it is desired to eliminate, but unsuitable for a like action upon the elements which it is desired to retain.

2. The process of producing low-carbon alloy-steel, which consists in first producing a ferro-alloy high in carbon and containing the desired proportion of the alloying metal with respect to iron, maintaining the prod-

uct in a molten condition at an approximately uniform elevated temperature in a refining chamber, and then subjecting the same to the action of an oxidizing gas having an oxygen pressure suitable for the oxidation of carbon but unsuitable for the oxidation of iron and the alloying metal.

3. The process of producing low-carbon alloy-steel, which consists in first producing a ferro-alloy high in carbon and containing the desired proportion of the alloying metal with respect to iron, maintaining the product in a molten condition at an approximately uniform elevated temperature in a refining chamber, mixing two or more gases in proportion to produce a gaseous agent having an oxygen pressure suitable, at the temperature at which the bath is maintained, for the oxidation of an element of the molten bath which it is desired to eliminate, but unsuitable for the oxidation of the elements which it is desired to retain, and subjecting the molten bath to said gaseous mixture.

4. The process of producing low-carbon alloy-steel, which consists in first producing a ferro-alloy high in carbon and containing the desired proportion of the alloying metal with respect to iron, heating a molten bath of such product in an electric furnace, maintaining the temperature of the bath below the point of excessive volatilization of the alloying metal, and subjecting said bath to the action of an oxidizing gas having an oxygen pressure suitable at the temperature selected for the oxidation of an element which it is desired to eliminate, but unsuitable for the oxidation of the elements which it is desired to retain.

5. The process of producing alloy-steel from an impure mixture containing iron and the alloying metal in the desired proportions, which consists in maintaining such mixture in a molten condition and in subjecting the molten bath to a gaseous oxidizing agent having an oxygen pressure, at the temperature of the bath, suitable for causing said gaseous agent to act as a reducing agent with respect to oxids of iron and of the alloying metal and at the same time to act as an oxidizing agent with respect to an element or elements which it is desired to eliminate from the bath.

6. The process of producing alloy-steel from a mixture containing a ferro-alloy high in carbon associated with sulfur and phosphorus, or either of them, as impurities, which consists in maintaining such mixture in the condition of a molten bath, melting a basic flux with said bath, and subjecting the molten bath to an oxidizing gas having an oxygen pressure suitable for the oxidation of an oxidizable element which it is desired to eliminate but unsuitable for the oxidation of the elements which it is desired to retain.

7. The process of producing alloy-steel from a mixture containing a ferro-alloy high in carbon associated with sulfur and phosphorus, or either of them, as impurities, which consists in maintaining such mixture, in the condition of a molten bath, melting a basic flux with said bath, and subjecting the molten bath to a gaseous mixture containing carbon dioxid in quantities regulated to produce, at the temperature of the bath, an oxygen pressure suitable for the oxidation of carbon but unsuitable for the oxidation of iron and the alloying metal.

8. The process of producing alloy-steel from a mixture containing a ferro-alloy high in carbon associated with sulfur, which consists in maintaining such mixture in the condition of a molten bath, melting a basic flux with said bath, subjecting the molten bath to gaseous reagents, suitable at the temperature selected for oxidizing carbon without attendant oxidation of iron or of the alloying metal and thereby producing in said flux conditions favorable for slagging off sulfur.

9. The process of producing alloy-steel from a mixture containing a ferro-alloy high in carbon associated with sulfur and phosphorus, or either of them, as impurities, which consists in maintaining such mixture in the condition of a molten bath, melting a basic flux with said bath, subjecting the molten bath to an oxidizing gas having an oxygen pressure suitable for the oxidation of carbon but unsuitable for the oxidation of iron or of the alloying metal, and then further subjecting the molten bath to a gas having less oxidizing and stronger reducing properties than said first mentioned gas.

10. The process of producing alloy-steels, which consists in first reducing suitable ores in the presence of carbon, then electrically heating the resultant high-carbon ferro-alloy to maintain the same in the condition of a molten bath having an approximately uniform predetermined temperature, and subjecting said bath to the action of a gas containing carbon dioxid in quantities suitable for the selective oxidizing action of said gas on carbon at said predetermined temperature but unsuitable for a like action on iron and the alloying metal.

11. The process of producing low-carbon alloy-steels, which consists in first producing a ferro-alloy high in carbon, electrically heating the product to a predetermined temperature below that for excessive volatilization of the alloying metal, and subjecting the electrically heated product to the action of an oxidizing gas suitable at said predetermined temperature for selective oxidizing action on carbon, but unsuitable for a like action upon iron and the alloying metal or metals.

12. The process of producing alloy-steel,

which consists in first producing a ferro-alloy high in carbon, maintaining the product in a molten condition at an approximately uniform elevated temperature in a refining chamber, subjecting the heated product to the action of a gaseous oxidizing agent having at said temperature an oxygen pressure suitable for an oxidizing action on the contained carbon but unsuitable for a like action upon the elements which it is desired to retain in the steel, and meanwhile regulating the pressure of the gases liberated in the refining chamber to control the volatilization of the alloying metal or metals.

13. The process of producing manganese-iron alloys directly from an alloy of iron and manganese having a high carbon content, which consists in maintaining the material in a molten condition at an approximately uniform predetermined temperature, and subjecting the molten material to the action of a gaseous oxidizing agent having at said temperature an oxygen pressure suitable for an oxidizing action on the oxidizable element or elements which it is desired to eliminate but unsuitable for a like action upon the elements which it is desired to retain.

14. The process of producing manganese-steel directly from spiegeleisen, which consists in maintaining said spiegeleisen at an approximately uniform predetermined temperature slightly above its melting point, and subjecting the molten material to the action of a gaseous oxidizing agent having at said temperature an oxygen pressure suitable for oxidizing carbon contained in the product under treatment but unsuitable for a like action on the elements which it is desired to retain in the steel.

15. The process of producing manganese-iron alloys directly from an alloy of iron and manganese having a high carbon content and containing oxidizable impurities and slag-forming impurities, which consists in maintaining such mixture in the condition of a molten bath, melting a basic flux with said bath, and subjecting the molten bath to an oxidizing gas having an oxygen pressure suitable for the oxidation of said oxidizable impurities but unsuitable for a like action upon iron and manganese.

16. The process of producing manganese-iron alloys directly from an alloy of iron and manganese having a high carbon content and containing oxidizable impurities and slag-forming impurities, which consists in maintaining such mixture in the condition of a molten bath, melting a basic flux with said bath, subjecting the molten bath to an oxidizing gas having an oxygen pressure suitable for the oxidation of said oxidizable impurities but unsuitable for a like action upon iron and manganese and then further subjecting the molten bath to a gas having

lesser oxidizing properties than said first mentioned gas.

17. The process of producing manganese steel directly from spiegeleisen containing 5 sulfur and phosphorus or either of them as impurities, which consists in maintaining such mixture in the condition of a molten bath, and subjecting the molten bath to an oxidizing gas having an oxygen pressure 10 suitable for the oxidation of the contained carbon but unsuitable for a like action upon iron or manganese, and subsequently subjecting said bath to the action of a reducing gas.
18. The process of refining a molten bath 15 of iron and manganese containing oxidizable impurities, which consists in subjecting said molten bath to a gaseous mixture having, at the temperature of the bath, oxidizing properties with respect to said impuri- 20

ties and non-oxidizing properties with respect to manganese.

19. The process of refining an alloy of iron and manganese having a high-carbon content and also containing sulfur or phosphorus, which consists in providing a molten bath of such alloy and a basic flux, and subjecting said molten bath to a gaseous mixture having, at the temperature of the bath, oxidizing properties with respect to carbon 25 and non-oxidizing properties with respect to iron and manganese.

In witness whereof, I, hereunto subscribe my name this second day of January, A. D., 1909.

ALBERT E. GREENE.

Witnesses:

GEORGE E. FOLK,  
ALFRED H. MOORE.

---